

June 3, 1924.

1,496,038

C. C. VENABLE

PROCESS OF ROLLING STEEL RINGS

Original Filed Feb. 8, 1921

2 Sheets-Sheet 1

Fig. 6.



Fig. 5.



Fig. 4.



Fig. 3.



Fig. 2.



Fig. 1.



Inventor

Charles C. Venable

By Church & Church

His Attorneys

June 3, 1924.

1,496,038

C. C. VENABLE

PROCESS OF ROLLING STEEL RINGS

Original Filed Feb. 8, 1921 2 Sheets-Sheet 2

Fig. 10.



Fig. 9.



Fig. 8.



Fig. 7.



Inventor

Charles C. Venable

By Church & Church

His Attorneys

## UNITED STATES PATENT OFFICE.

CHARLES C. VENABLE, OF WASHINGTON, DISTRICT OF COLUMBIA, ASSIGNOR, BY MESNE ASSIGNMENTS, TO THE WELDLESS ROLLED RING COMPANY, A CORPORATION OF OHIO.

## PROCESS OF ROLLING STEEL RINGS.

Application filed February 8, 1921, Serial No. 443,367. Renewed November 13, 1923.

To all whom it may concern:

Be it known that I, CHARLES C. VENABLE, a citizen of the United States, residing at the city of Washington, District of Columbia, have invented certain new and useful Improvements in Processes of Rolling Steel Rings; and I do hereby declare the following to be a full, clear, and exact description of the same, reference being had to the accompanying drawings, forming part of this specification.

This invention relates to the manufacture of metal annular bodies or rings by the rolling of a cast or forged blank of approximately the same weight as the finished ring but of relatively smaller diameter.

The object of the present invention is to provide a process whereby it is possible to roll small finished rings of irregular shape from annuli. A further object of the invention is to provide a process, the use of which will eliminate the formation of annular grooves on the various faces of a rolled ring, such grooves or draws usually occurring on the wall faces of the ring.

A further object of the invention lies in the provision of a process in the practice of which each pressure point on the top or bottom face of the biscuit will be in the same plane as the wall face of the corresponding reentrant angle of the finished ring.

It has long been known that metals whether of uniform structure such as copper or aluminum or of fibrous structure such as iron or steel may be greatly elongated by being passed through a pair of driven rolls, the space between such rolls being less than the thickness of the ingot or blank, and that by making suitable indentations in one or the other or both of the rolls various forms of straight material may be obtained, such rolled sections being for example, railway rails, I-beams, angles, channels, etc.

It has also been old to roll large annular bodies such as locomotive tires by having an outer roll formed as a separable mold and having the inner roll which is mounted on a movable axis, drive the plastic metal into the cavity in the larger roll, so that when

the annular body is completely formed, it will exactly fill the mold, but as far as I know no practical process has ever been known that would permit the rolling of an annular body of steel between a mandrel and a roll where the blank was free to expand lengthwise of the axis of the roller, although small rings of rectangular cross section have been rolled to a similar rectangular cross section with the formation on both wall faces of draws which are eliminated by machining the rolled ring to size, which is invariably less than the distance between the deepest portions of the two draws.

Where two rolls are used, which rotate upon constantly parallel axes, it will be apparent that the side spread of a piece of metal whether annular or straight does not depend in any way upon the width of the material being rolled, but is dependent upon the original thickness of the metal blank, the angle of pressure and the distance between the two rolls, which distance is commonly known as the "pass." The spreading may thus be kept at a very low figure by having a relatively large pass and a low angle of pressure, annular rolling being particularly suitable to small side expansion as the angle of approach may be kept at a very low figure, say three degrees or less, and the angle of pressure will be correspondingly low as it is a function of the angle of approach.

In rolling rings of copper or aluminum the metal has been found to flow so as to take care of slight irregularities, but with fibrous materials such as iron and steel, the strength of the metal is very different with the grain and transversely thereof, and for this reason it has been found practically impossible to successfully roll annular shapes of iron or steel, save where the finished shape was rectangular in cross section, and even in this formation a very considerable amount of metal is required to be machined off from the rolled ring.

In view of the enormous cost of labor at the present time, it has become more and more desirable to forge steel blanks and to roll them out to finished shape for such

forms as internal ring gears, rings for ball bearings, bevel gears, etc., but the difficulty has always been met that in rolling such shapes deep annular draws have been formed in practically all of the wall faces of the rolled ring and frequently in one or more of the side faces as well.

A further and more serious difficulty has been the formation of deep weakening draws in all of the reentrant angles to such extent that the cost of a rolled ring of this form is greater than the cost of casting the piece and machining it, although it is true that a rolled ring machined down to proper size is materially better than a ring obtained by casting. As far as I know however, the rolling of small steel rings of irregular shape has never been performed, except experimentally, and then only in the works 20 of the company with which I am connected.

Careful study of the imperfections in the rolled rings indicates that in irregular shapes such as a flanged ring, the flange being relatively small will cool considerably quicker during the rolling process than will the body of the blank, thus causing almost invariably a draw on both wall faces of the flange, as well as a similar imperfection in the reentrant angle where the flange joins 30 the body, the latter being caused by the drawing of metal from the heated body to the relatively cooler flange.

Other annular concavities or draws are formed elsewhere on the rolled ring, normally occurring on the wall faces of the body, probably due to the spreading of the metal on the inner or bottom face against the mandrel and on the outer or top face against the roll, each causing the metal to 40 flow in a direction parallel to the axis of the rolls, that is, sideways of the cross section of the blank. During this action, the central strata of the metal between the two rolled faces is slipping backward in the direction 45 of rotation of the rolls, while the outer and inner faces are being pushed forward, thus causing a backward slippage of the central portion of the body due to the difference in length between the outer and inner faces, 50 which as might be expected, causes end grooves or draws in each of the wall faces of the rolled ring.

In order to clearly understand the process to be described it is well to define the various terms used in the art. The blanks are invariably annular with a central hole known as the bore which is the smallest diameter of the hole. The largest diameter of the blank taken as a whole is the overall diameter and half of the difference between the overall diameter and the bore diameter is called the radial thickness of the blank. Any plane passing through the axis of the blank will cut the blank or biscuit forming a cross section known as a projection wall section, the

greatest height of which is the radial thickness and the dimension at right angles thereto is known as the axial width of the blank.

The outer faces of the blank are called the top faces to distinguish them from the inner or bottom faces which contact with the mandrel while the top faces contact with the movable roll. The side faces are called wall faces, that part of the wall face nearest to the top face being known as the outer wall face, while the one offset therefrom nearest to the axis of rolling is the inner wall face. The side of the blank nearest to the rolling machinery is known as the rear of the blank, while the side that faces in the same direction as the smaller diameter of the mandrel is the front of the blank. The width of the draw is the greatest dimension of the draw measured radially and in a wall section, for example, it is taken parallel to the radial thickness of the blank while the depth of the draw is measured at right angles thereto in accordance with the usual meaning of the term. The draft is the angle of relief formed on the side or wall and is measured in terms of degrees of inclination, usually 3, 5, or 7. The length of draft is measured along the longer leg of the angle considered as a right triangle and the depth is measured at right angles thereto or along the shorter leg of such triangle. The length of the draft is determined by the diameter of the finished ring at that point and it increases proportionately with such diameter, that is the greater the amount of 100 rolling required, the greater the length of the draft and consequently the greater the depth of the draft as well.

In the drawings,—

Fig. 1 is a midsection of an annulus;

Fig. 2 is a similar view of the ring as rolled from the annulus illustrated in Fig. 1;

Fig. 3 is a midsection of an incorrectly formed blank;

Fig. 4 is a midsection of the rolled section obtained from the blank of Fig. 3;

Fig. 5 is a midsection of a correctly formed blank;

Fig. 6 is a midsection of a finished ring ready for machining into an internal ring gear;

Fig. 7 is a section of a forged ring blank;

Fig. 8 is a similar section of the rolled ring obtained therefrom and suitable for machining into a driving bevel gear; and

Fig. 9 is a diagrammatic view of a "set-up" for rolling the ring shown in Fig. 6.

Fig. 10 is a section of a blank for rolling a ring of rectangular cross section.

In Figure 1 is shown an annulus consisting of a body 11 having an outwardly extending flange 12, the latter having a top face 13 beveled at a forging angle of 5°,

while the body has a top face 14 beveled at a somewhat greater angle. The bottom faces 15 and 16 are similarly beveled at angles of 5° and 7° but the side or wall faces are left flat to correspond with the wall faces of the ring desired. Upon rolling this blank, however, the resulting ring, as shown in Figure 2, is found to be defective due to the deep draws 20 and 21 formed at the apex of the two 10 reentrant dihedral angles and by the formation of the annular grooves 22 and 23 in the front and rear wall faces.

The faulty shape of the rolled ring is due to improper design of the forged annulus. 15 In the annulus the volume of the flange being considerably less than the volume of the body causes a higher percentage of heat reduction in the flange to that in the body, so that during the rolling process the flange in 20 cooling first has its wall faces chilled, and then since the great mass of the body is still hot, metal is drawn from the center of the relatively cool flange, thereby developing the concave faces 20 and 23 on the flange and 25 also the similar draw 21 at the junction of the flange and body. The draw 22 appears to be directly due to the spreading of the metal on the bottom face 16 and the top face 14 of the body in a longitudinal direction 30 causing a simultaneous backward slipping of the central portion of the body, due to the difference in the peripheral length of faces 14 and 16, this condition not only forming the draw 22, but likewise contributing to the 35 formation of the annular concavity 21.

In the experimental work in developing this invention, it was found that a considerable shortening of the flange, (see Fig. 3), a reduction to one-third its volume, and the 40 relieving of the face C' D' by a draft of 5° the entire distance from C' to D', removed entirely the draw 20, since this reduction maintained the heat in the flange for a considerably longer time, and also allowed for 45 the formation of the flange with a minimum contact with the upper roll. The draft angle of face 15 which had previously been 7° was now changed to 20° which reduced the contact in rolling, but was not sufficient relief 50 to eliminate the draw of the metal at 21; but with an increase of draft (as shown in Fig. 5) in this counterbore to 45° the draw 21 was entirely eliminated, and with the formation of a relief angle or draft at the 55 corner B' of 7° the finished ring was found to be perfect in all respects, the blank now having the form shown in Figure 5, wherein the outer top face B—C is sloped at an angle of 5° which is the present normal drop 60 forging top face practice; the inner top face D—E is provided with a draft of 7° owing to its coming first into contact with the top roll 30; the front inner wall of face F—G is flat except for the relief E—F of 7°; the 65 bottom face H—G of the body is of 7° draft

which is the usual drop forging practice; the inner wall face K—H is flat, but the rear bottom face M—K is relieved to the extent of 45° which allows the rear wall face A—M to be flat.

Referring now particularly to Figure 9 showing the set-up for rolling the internal gear shown in Fig. 6, the blank or annulus 31 is placed upon the mandrel 32 and is pushed rearwardly until the inner rear wall 70 face H—K abuts the shoulder 33 of the mandrel at which time also the rear wall face A—M will be in contact with the flange 34 which revolves with the mandrel and may be an integral part thereof if so desired. 80 The top roll 30 is now lowered into contact with the blank, the rounded corner 35 of the top roll striking approximately at the point D which lies in the plane of the finished front outer wall face of the flange of the 85 gear while the similar rounded point 36 of the mandrel likewise strikes approximately at the point K which lies in the plane of the rear outer wall of the body. It is quite essential that these conditions should obtain; that is, that the plane of the shoulder of the mandrel should correspond with the plane of the corresponding wall face of the finished ring and that the plane of the shoulder of the roll should correspond with the 90 plane of the corresponding wall face of the finished ring. If this were not true, the blank will be given a torsional strain which will create a stress and consequent weakness in the rolled section. It should be borne 95 in mind, however, that where either the roll or the mandrel is rounded as is the case in Figure 9, that the point of the shoulder should be considered as the meeting point of the shoulder and periphery as if they met in 100 a sharp angle.

The sleeve 37 is mounted to revolve in a reciprocating carriage and during the rolling operation the carriage is moved towards the mandrel which enters a recess in the 110 sleeve with the latter in very close proximity to, but not actually touching the outer side of the top roll. As the top roll is brought nearer and nearer to the mandrel the circumference of the blank is increased 115 and the rolling is continued until the blank, which is now the finished ring, is in contact with the three faces of the top roll, the four faces of the mandrel and the single face of the sleeve at which time the diameter of the ring will be the correct size since no draws are formed, due to the presence of the relief angles. Without these drafts, draws would be formed no matter how great the pressure 120 of the top roll and sleeve and it will be found that where these draws are present there will be less area in the cross section of the completed ring and consequently when the top roll is lowered to its extreme point 125 the diameter of the ring will be considerably 130

greater than the required diameter, for the reason that the metal displaced by the draw has simply added to the periphery of the ring, that being the only point of outlet for 5 the excess metal. It will be noted that there is no relief at the point G. This has been found unnecessary in practice where the amount of rolling is not great and the distance E—G not excessive. The provision of 10 a relief at this point, however, would actually aid in making the face F—G slightly smoother, but as stated, in practice it is unnecessary for the reason that an appreciable amount of machining is desirable, say a sixteenth of an inch and that if the finished blank were reduced to within a thirty-second or less of the ground size, the operation would be more expensive, due to the length 15 of time it would take to secure the perfect set in the grinding machine.

Figure 7 shows a biscuit or blank correctly designed for rolling the rear axle drive gear shown in Figure 8. The faces 43 and 44 are slightly beveled to permit rolling and the corresponding faces 45 and 46 of the blank preserve the chosen angles. The faces 47, 48, 49 and 50 are exactly parallel to the ground finished faces of the gear and the corresponding faces in the blank 51, 30 52, 53 and 54 exactly correspond in direction to the faces of the finished ring. As will be noted from the dotted lines in Figure 7 representing the "set-up," the top roll and the mandrel are both grooved to the 35 proper shape of the finished ring and no side pieces such as the flange 34 and the sleeve 37 are required. There is no tendency for the metal to squeeze out between the mandrel and top roll where the faces 40 are correctly beveled to the finished shape unless excess metal is present.

It will be understood that the annulus must contain the same weight of metal as the finished ring but when an annulus has 45 been designed for any size ring or annulus the change to a different size presents no difficulty whatsoever since to roll a larger diameter ring, for example, from the blank of Fig. 7, it is merely necessary to draw a 50 cross section of the blank on a sheet of paper and divide such cross section by a line parallel to the axis of rolling, such a line being 41 of the figure. Now by splitting the cross section on this line and by inserting a

rectangular section between the two severed portions of the cross section such rectangle being of the same length as the cross section is wide and being of such area that the volume of metal corresponding to such area shall be the required additional weight 60 of metal a new cross section is formed which will be the accurate cross section of a blank which will roll the new size larger diameter ring. To roll a smaller size ring the same procedure is followed, but in this case after 65 severing the cross section a rectangular area is removed such; for example, as that between the lines 41 and 42 of Fig. 7. By now joining the two remaining sections the new cross section is formed. It will be 70 noted that neither of these two operations affects any of the angles of the annulus since the wall faces of the added or subtracted area are flat, that is, they are normal or perpendicular to the axis of rolling. 75

What I claim is:

1. The art of eliminating draw in a rolled ring which consists in taking an annular blank having its wall faces relieved by the provision of drafts on each edge of said faces and rolling the blank circumferentially.

2. The art of eliminating draw in a rolled ring which consists in taking an annular blank having a body and a peripheral flange with an obtuse reentrant angle between the flange and the body and rolling said blank circumferentially.

3. The art of eliminating draw in a rolled ring which consists in taking an annular blank having a body and an outwardly extending peripheral flange with a reentrant angle between said flange and body, rendered obtuse by relieving the wall face forming one wall of said reentrant angle 90 and rolling said blank circumferentially.

4. The art of eliminating draw in a rolled ring which consists in taking a blank of smaller diameter than the size of the finished ring but of substantially equal weight, 100 and having its outer and inner faces parallel to that desired for the finished faces of the rolled ring and in rolling said blank circumferentially to force the excess metal in the center of the blank to form the increased diameter desired in the finished ring. 105

CHARLES C. VENABLE.